

Oct. 8, 1940.

M. C. KUMNICK ET AL

2,217,171

STIFFENING MEMBER FOR SHOES AND THE LIKE

Filed Sept. 8, 1938



*Fig. 1*

*Fig. 4*



*Fig. 2*



*Fig. 3*

Miles C. Kumnick INVENTORS  
Quentin L. Quinlivan

BY

J. M. Castle Jr.  
ATTORNEY

## UNITED STATES PATENT OFFICE

2,217,171

STIFFENING MEMBER FOR SHOES AND THE  
LIKE

Miles C. Kumnick, Kearny, and Quentin L. Quinlivan, Arlington, N. J., assignors to The Celastic Corporation, Wilmington, Del., a corporation of Delaware

Application September 8, 1938, Serial No. 228,924

6 Claims. (Cl. 36—77)

This invention relates to heat-softening stiffening members for shoes, and the like, and, more particularly, to those members ordinarily known as box toes and counters made from a homogeneous plastic composition as distinguished from the more common type made from a fabric impregnated with a thermoplastic substance.

In ordinary shoe making practice, stiffening members are incorporated into the construction while in a soft and pliable condition which permits of their being pulled into shape over the last. These members fall into two classes with respect to the method of softening them, the solvent softening class, which are soaked in or saturated with a solvent which softens them, and the heat softening class which are made pliable by heating, usually in a "steamer," to about 80—100° C. This latter is a simpler and preferable technique.

Of the rigid heat softening type of shoe stiffener, most of those in commercial use comprise a fabric impregnated with a thermoplastic substance. Solid sheeting of thermoplastic material has not been used heretofore as a heat softening stiffener because it has been impossible to meet, in a single material, the essential requirements that the sheeting become adequately softened for fabrication at 80—100° C. and that it resist distortion by heat at the temperatures of service. In so far as solid thermoplastic sheeting, e. g., a pyroxylin plastic, has been used for box toes, and the like, it has been softened by solvent rather than by heat.

The present invention relates to stiffeners of this solid type which are capable of being adequately softened by steamer temperatures while adapted to resist distortion at temperatures of service.

The characteristics which should be possessed by such stiffening members, particularly the box toes used in the construction of dress shoes, have been recognized for many years by the trade but the materials heretofore proposed for use for this purpose have fallen short of presenting complete combinations of all of the essential features from both the standpoint of fabrication and service.

A stiffening member should be resilient and strong so that if, distorted or dented by pressure, it will resume its original shape upon release of the pressure and not be weakened thereby. Such stiffening members also should not be subject to deterioration or distortion with age nor be damaged by complete immersion in water. From the standpoint of fabricating technique, the material for the stiffener should be of a form and

character which will not introduce undue expense and operating difficulties in the construction of the shoe. Its heat softening characteristics must be such that it softens adequately in the ordinary "steamer" and retains its softness long enough to be formed over the last.

It is further desirable that, with a minimum of auxiliary treatment to that end, the shoe stiffener should be capable of cementing itself, or of being cemented to adjacent layers in the construction of the shoe so that the latter will have a maximum stability and derive from its adhesion to the box toe a degree of protection against wrinkling and creasing of one layer over the other. Still further, it is desirable in many cases that a stiffener be of light color so as to impart no undesirable dark undertone to light colored translucent fabrics with which it is used in fancy shoes.

An object of the present invention is to provide a non-reinforced heat softening material for stiffening elements in shoes, and the like, which shall present a maximum number of the desirable characteristics outlined above and shall be free from the defects exhibited by materials heretofore proposed for this purpose. A further object is to provide such material for stiffening elements of shoes which shall be easily and economically incorporated into the structure of the shoe, shall have strength and resilience to resist distortion and to regain its original shape if distorted, which shall not be subject to warpage or other deterioration with age and service of the shoe, which shall lend itself readily to adhesion with adjacent layers in the construction of the shoe and which shall be capable of being formed and incorporated into the structure of the shoe so as not to be objectionably visible from the outside of the latter. A still further object is to provide a stiffening material which shall have the advantage of sightlessness and thus be adapted to serve as an externally visible member in the construction of the shoe. Other objects of the invention will be apparent from the description given hereinafter.

The above objects are accomplished according to the present invention by making stiffening members for shoes of a plastic composition comprising ethyl cellulose and a plasticizer in an amount ranging from 17—67 parts, by weight, per 100 parts of ethyl cellulose.

It has been discovered that ethyl cellulose suitably plasticized within the range given above provides a heat softening plastic which fulfills satisfactorily the vital characteristics of an ac-

ceptable shoe stiffener of the type herein considered. More specifically, in addition to having the other properties requisite in a plastic for use as a shoe stiffener, suitably plasticized ethyl cellulose gives a stiffening member for use in shoes that is readily softened in the conventional "steamer" and which is so resilient and strong at temperatures of service in the shoe that it not only imparts the required support to the leather or fabric used in the shoe but, if distorted or dented by pressure, it will resume its original shape upon release of the pressure and not be weakened thereby. These ethyl cellulose compositions are adapted to be worked up into beveled box toe blanks and similar shoe stiffener blanks by processes of thermoplastic molding and particularly by injection molding.

It has further been discovered that, by employing as the plasticizer for the ethyl cellulose a mixture of a non-exuding plasticizer and an exuding plasticizer, the latter amounting to at least 10% of the combined weight of ethyl cellulose and plasticizers, a composition results which gives a stiffening member that is adhesive at the temperature of lasting. Further, it has been found that the compositions of the present invention may include up to 50%, by weight of the total composition, of a compatible extender although it is preferred not to employ a compatible extender in excess of 25% of the total weight of the composition.

In Examples I to XI given hereinafter are illustrated specific embodiments of the invention wherein the ethyl cellulose is plasticized with non-exuding plasticizers alone. The non-exuding plasticizers are defined, for the sake of definiteness, as those plasticizers for ethyl cellulose which are compatible therewith in proportions up to at least 67 parts per 100 parts of ethyl cellulose without being subject to exudation from the resulting plastic when it is heated to temperatures up to 200° C.

These plasticizers serve primarily to enhance the resilience and strength of the material and include the following:

- 45 Butoxy ethyl stearate
- Butyl stearate
- Camphor
- Castor oil
- 50 Diamyl adipate
- Diamyl phthalate
- Dibutyl phthalate
- Dibutyl sebacate
- Dibutyl tartrate
- 55 Diethyl phthalate
- Dimethoxyethyl phthalate
- Diphenyl mono-xenyl phosphate
- Diphenyl phthalate
- Dicresoxy diethyl ether
- 60 Mixture of alcohols of higher molecular weight sold under the trade-name "Lorol"
- Mixture of phthalic acid esters of alcohols of 6, 7, and 8 carbon atoms
- 65 Monophenyl di-o-xenylphosphate
- Octadecane diol diacetate
- Palmitic acid
- Para-coumarone para-indene resins of liquid type, such as those sold under the name "Cumar"
- Tributyl phosphate
- 70 Tricresyl phosphate
- Tri-o-xenyl phosphate
- Triphenyl phosphate

Those skilled in the art will understand that by the term "ethyl cellulose" as used herein, is

meant the high substituted, organic solvent soluble type generally adapted for use in the plastics field as distinguished from the low substituted type of difficult solubility in organic solvents, if soluble at all, and primarily adapted for uses outside of the plastics field.

In Example I given hereinafter reference is made to the accompanying drawing wherein:

Fig. 1 is a plan view of a box toe blank of conventional form;

Fig. 2 is a section on the line 2—2 of Fig. 1;

Fig. 3 is a section similar to Fig. 2 of a blank of different shape; and

Fig. 4 is a plan view of a blank of still another shape.

The following examples, wherein all parts are given by weight unless otherwise indicated, illustrate specific embodiments of the invention:

*Example I.*—A homogeneous sheeting composition of 100 parts of ethyl cellulose and 33 parts of a mixture of phthalic acid esters of alcohols of 6, 7, and 8 carbon atoms is made by any convenient manner known in the art. By means of a suitable molding die, portions of this sheeting are shaped by the ordinary technique of thermoplastic molding to form blanks of the form indicated in Figs. 1 and 2. The bevel 11 ordinarily provided by skiving is thus provided by molding.

The blank thus made is heated to a temperature of 80-100° C. on a steamer and is thereby made limp, pliable, and capable of being considerably stretched without being torn. While in this limp condition, which is retained for a period of at least 15 seconds, the blank is inserted in the usual manner between a lining and a leather upper and pulled to shape over the toe of a last. The gathered edge of the blank is nailed to the sole of the last. Construction of the shoe proceeds in the usual manner, including the operation of steaming, or other suitable means of completing the lasting, which fails to distort or wrinkle the stiffening member.

Upon completion of the shoe, this stiffened toe, even though of less or no greater than ordinary thickness, has sufficient rigidity to resist ordinary distorting forces and, if distorted by heavy pressure or a sharp blow, such as that of a hammer, it will return to its original shape and be neither cracked nor weakened by such treatment. Further, it is not subject to distortion through prolonged severe service wherein it is subject continually to temperatures of the order of 35-45° C. and to high humidity or actual contact with moisture.

In the further examples the method of preparation and the manner of use may be as in Example I. It will be evident to those skilled in the art that the shaped blank with its bevel or scarf, or with other variations from flat sheet form such as general non-uniformity of thickness for the purpose of locally enhancing strength or rigidity as in the shape illustrated in Fig. 3, may be molded not only by compression molding of a continuous preliminary blank cut from sheet or slab material but also by compression molding of the same composition in the discontinuous form of a molding powder; also, that it may be formed by the equally well known technique of injection molding or by the modification of the latter known as transfer molding. It will be evident that by so forming the blanks it is feasible to fabricate blanks of irregular shapes such as that shown in Fig. 4 to which it would be expensive and difficult, if not altogether impossible, to impart the

desired bevel such as 12 in Fig. 4, by skiving machines.

*Example II*

|                                                                            | Parts |
|----------------------------------------------------------------------------|-------|
| Ethyl cellulose                                                            | 100   |
| Mixture of phthalic acid esters of alcohols of<br>6, 7, and 8 carbon atoms | 54    |

*Example III*

|                     |     |
|---------------------|-----|
| Ethyl cellulose     | 100 |
| Tricresyl phosphate | 54  |

*Example IV*

|                     |     |
|---------------------|-----|
| Ethyl cellulose     | 100 |
| Triphenyl phosphate | 33  |

*Example V*

|                     |     |
|---------------------|-----|
| Ethyl cellulose     | 100 |
| Tricresyl phosphate | 33  |

*Example VI*

|                                                                            |     |
|----------------------------------------------------------------------------|-----|
| Ethyl cellulose                                                            | 100 |
| Mixture of phthalic acid esters of alcohols of<br>6, 7, and 8 carbon atoms | 43  |

*Example VII*

|                  |     |
|------------------|-----|
| Ethyl cellulose  | 100 |
| Diamyl phthalate | 43  |

*Example VIII*

|                                                                            |     |
|----------------------------------------------------------------------------|-----|
| Ethyl cellulose                                                            | 100 |
| Octadecanediol diacetate                                                   | 28  |
| Mixture of phthalic acid esters of alcohols of<br>6, 7, and 8 carbon atoms | 14  |

*Example IX*

|                                                                            |      |
|----------------------------------------------------------------------------|------|
| Ethyl cellulose                                                            | 100  |
| Mixture of phthalic acid esters of alcohols<br>of 6, 7, and 8 carbon atoms | 17.5 |

*Example X*

|                                                                            |     |
|----------------------------------------------------------------------------|-----|
| Ethyl cellulose                                                            | 100 |
| Mixture of phthalic acid esters of alcohols of<br>6, 7, and 8 carbon atoms | 67  |

*Example XI*

|                    |     |
|--------------------|-----|
| Ethyl cellulose    | 100 |
| Tributyl phosphate | 33  |

50 Compositions of the type illustrated by Examples I to XI do not possess adhesive characteristics when softened by dry heat or by steam. It has been found that the replacement of part or all of the non-exuding plasticizer in compositions 55 of this type by a plasticizer of exuding character confers upon the composition a character of adhesiveness when hot, so that adjacent fabric in the structure of the shoe may thereby be caused to adhere firmly to the stiffening member.

60 Plasticizers designated as exuding, for the purpose of the present specification, are characterized by being compatible with ethyl cellulose in that in proportions up to about 50 parts per 100 parts of ethyl cellulose they do not exude more 65 than slightly, at ordinary temperatures, from a plastic of ethyl cellulose with which they have been homogeneously incorporated, but are driven to the surface of the plastic upon the application of heat at temperatures above the useful softening 70 temperature of the plastic.

Upon heating a blank containing such a plasticizer in suitable proportions to such a temperature that it becomes adequately softened for use, e. g., to a temperature of from 80 to 100° C., a liquid comes to the surface of the material, and

if the blank, while in this condition, be inserted in the shoe structure and pulled over the toe of a last, the ordinary pressure applied incidental to this operation causes the formation of a bond between the fabric and the ethyl cellulose stiffener. 5 The minimum proportion of exuding plasticizer which imparts a useful adhesiveness to the composition is ten percent of the combined weight of the ethyl cellulose and plasticizer used.

Among the exuding plasticizers particularly 10 adapted for use in the present invention are stearic acid and a mixture composed chiefly of primary, straight chain saturated aliphatic alcohols of 16, 17, and, predominantly, 18 carbon atoms derived from hydrogenated cocoanut oil. 15 This latter mixture is a commercial product susceptible to some fluctuation in the proportions of its components; it will be referred to hereinafter as "eighteen-carbon" alcohol.

Examples of compositions containing exuding 20 plasticizer in proportions sufficient to confer useful adhesive properties are given in Examples XII to XX:

*Example XII*

|                         | Parts |
|-------------------------|-------|
| Ethyl cellulose         | 100   |
| Triphenyl phosphate     | 21.5  |
| Eighteen-carbon alcohol | 21.5  |

*Example XIII*

|                                                                            |     |
|----------------------------------------------------------------------------|-----|
| Ethyl cellulose                                                            | 100 |
| Mixture of phthalic acid esters of alcohols of<br>6, 7, and 8 carbon atoms | 31  |
| Eighteen-carbon alcohol                                                    | 23  |

*Example XIV*

|                                                                            |     |
|----------------------------------------------------------------------------|-----|
| Ethyl cellulose                                                            | 100 |
| Mixture of phthalic acid esters of alcohols of<br>6, 7, and 8 carbon atoms | 14  |
| Eighteen-carbon alcohol                                                    | 29  |

*Example XV*

|                         |     |
|-------------------------|-----|
| Ethyl cellulose         | 100 |
| Tricresyl phosphate     | 23  |
| Eighteen-carbon alcohol | 31  |

*Example XVI*

|                                                                            |     |
|----------------------------------------------------------------------------|-----|
| Ethyl cellulose                                                            | 100 |
| Mixture of phthalic acid esters of alcohols of<br>6, 7, and 8 carbon atoms | 25  |
| Stearic acid                                                               | 23  |

*Example XVII*

|                                                                            |     |
|----------------------------------------------------------------------------|-----|
| Ethyl cellulose                                                            | 100 |
| Mixture of phthalic acid esters of alcohols of<br>6, 7, and 8 carbon atoms | 50  |
| Eighteen-carbon alcohol                                                    | 55  |

*Example XVIII*

|                                                                            |     |
|----------------------------------------------------------------------------|-----|
| Ethyl cellulose                                                            | 100 |
| Mixture of phthalic acid esters of alcohols of<br>6, 7, and 8 carbon atoms | 50  |
| Stearic acid                                                               | 15  |

*Example XIX*

|                                                                            |     |
|----------------------------------------------------------------------------|-----|
| Ethyl cellulose                                                            | 100 |
| Mixture of phthalic acid esters of alcohols of<br>6, 7, and 8 carbon atoms | 65  |
| Eighteen-carbon alcohol                                                    | 5   |

*Example XX*

|                                                                            |     |
|----------------------------------------------------------------------------|-----|
| Ethyl cellulose                                                            | 100 |
| Mixture of phthalic acid esters of alcohols of<br>6, 7, and 8 carbon atoms | 5   |
| Stearic acid                                                               | 15  |

If desired, the non-exuding plasticizer may be omitted altogether and one or a mixture of the

exuding plasticizers may be used as the plasticizer, as indicated in Examples XXI to XXIII. This, however, is not preferred, as the resulting compositions do not have quite the resilience and strength of those containing non-exuding plasticizer:

*Example XXI*

|                            | Parts |
|----------------------------|-------|
| Ethyl cellulose            | 100   |
| 10 Eighteen-carbon alcohol | 40    |

*Example XXII*

|                 | Parts |
|-----------------|-------|
| Ethyl cellulose | 100   |
| 15 Stearic acid | 40    |

*Example XXIII*

|                            | Parts |
|----------------------------|-------|
| Ethyl cellulose            | 100   |
| 20 Eighteen-carbon alcohol | 20    |
| Stearic acid               | 20    |

20 The mixtures of ethyl cellulose and plasticizer may be modified by the addition of compatible extenders, primarily for the purpose of reducing the materials cost of the mixtures. The term 25 "extenders" is used herein to characterize substances which may be homogeneously incorporated with ethyl cellulose and the plasticizers already mentioned, but which possess only very weak plasticizing power, if any, and which, in the 30 proportions used, do not exude more than slightly from the plastic.

Suitable extenders include the following: 35 Light-colored petroleum asphalt, such as that sold under the name "Albinalt"

Beeswax

Candelilla wax

Carnauba wax

Cetyl alcohol

Chlorinated diphenyl, such as that sold under the name "Aroclor".

40 Hydrogenated castor oil, such as that sold under the name "Opalwax".

Japan wax

Mineral rubber ("Gilsonite")

Montan wax

45 Oleic acid

Para-coumarone para-indene resins, such as those sold under the name "Cumar," of both solid and liquid types

Rosin

50 Spermaceti

Stearin pitch

Tallow

55 In mixtures containing extenders the ratio of ethyl cellulose to plasticizer is maintained in the range already set forth, and the percentage of extender in the mixture of ethyl cellulose, plasticizer, and extender, is not in excess of 50 percent, while about 25 percent is preferred as the 60 limit.

65 Compositions containing such extenders are illustrated by Examples XXIV to XXX.

*Example XXIV*

|                                                                         | Parts     |
|-------------------------------------------------------------------------|-----------|
| Ethyl cellulose                                                         | 50 (100)  |
| Mixture of phthalic acid esters of alcohols of 6, 7, and 8 carbon atoms | 20.5      |
| 70 "Cumar" resin of fusing point (ring and ball) 110° C.                | 20.5 (41) |

*Example XXV*

|                             | Parts      |
|-----------------------------|------------|
| Ethyl cellulose             | 62.5 (100) |
| 75 Tricresyl phosphate      | 12.5 (20)  |
| Light-colored petroleum wax | 25         |

*Example XXVI*

|                                                                         | Parts     |
|-------------------------------------------------------------------------|-----------|
| Ethyl cellulose                                                         | 63 (100)  |
| Mixture of phthalic acid esters of alcohols of 6, 7, and 8 carbon atoms | 21        |
| Carnauba wax                                                            | 16 } (33) |

*Example XXVII*

|                                                                         | Parts       |
|-------------------------------------------------------------------------|-------------|
| Ethyl cellulose                                                         | 70 (100) 10 |
| Mixture of phthalic acid esters of alcohols of 6, 7, and 8 carbon atoms | 15          |
| Hydrogenated castor oil                                                 | 15 (21.5)   |

*Example XXVIII*

|                                                                         | Parts       |
|-------------------------------------------------------------------------|-------------|
| Ethyl cellulose                                                         | 55 (100)    |
| Mixture of phthalic acid esters of alcohols of 6, 7, and 8 carbon atoms | 15          |
| Chlorinated diphenyl                                                    | 15 } (27.5) |
| Rosin                                                                   | 15          |

*Example XXIX*

|                                                                         | Parts       |
|-------------------------------------------------------------------------|-------------|
| Ethyl cellulose                                                         | 70 (100) 25 |
| Mixture of phthalic acid esters of alcohols of 6, 7, and 8 carbon atoms | 15 } (21.5) |
| Chlorinated diphenyl                                                    | 15          |

*Example XXX*

|                                                                        | Parts     |
|------------------------------------------------------------------------|-----------|
| Ethyl cellulose                                                        | 55 (100)  |
| Mixture of phthalic acid esters of alcohols of 6, 7 and 8 carbon atoms | 35 } (64) |
| Montan wax                                                             | 10 } 35   |

It will be understood that the above examples are merely illustrative and that the invention broadly comprises employing properly plasticized ethyl cellulose in nonreinforced stiffening members for shoes. While numerous specific examples of ethyl cellulose compositions have been given, as well as the range of proportions of plasticizers, the optimum composition using any particular plasticizer, or combination of plasticizers, for a desired purpose will involve some preliminary testing as those skilled in the art will appreciate.

The ethyl cellulose compositions of the present invention may be fabricated into blanks for box toes of ornamental character. Such stiffeners are adapted to be used without the usual outer covering of leather or fabric, and thus to be visible as an ornamental element of the shoe. Those stiffeners of translucent or transparent character are likewise adapted to be used without lining to provide an ornamental variant of ordinary shoe construction useful in obtaining novel effects in women's fancy shoes.

Many of the compositions set forth in the examples are approximately colorless and transparent and can be used unchanged for these bare or partially covered box toes. Or they may be colored to desired hues and made translucent or opaque if preferred. Preferably, box toe elements of this type will be made from compositions free from exuding plasticizers and free from extenders.

The present invention is not only applicable to stiffening members for box toes but is also applicable to stiffening members used as counters in shoes. The materials of the present invention, supplied in the form of sheeting or blanks, can be shaped into counters by the technique of heat softening followed by swaging in a cold mold or

molding powders of plasticized ethyl cellulose may be molded directly into shaped counters.

Not only are the compositions of the present invention suitable for shoe stiffeners but they 5 may also be used where similar requirement of toughness, resilience, water-proofness, and the like are required, particularly in articles of arched shape and including protective equipment for sports and games, arch supports, artificial 10 limbs, and the like.

An advantage of the present invention is that it provides shoe stiffeners of marked superiority over materials heretofore available in the preferred heat softening class and that box toes of 15 the herein described ethyl cellulose composition, with no support or reinforcement as woven fabric, felt, wire netting, loose fiber, and the like, are superior to heat softening stiffeners heretofore proposed even when so supported or reinforced. A further advantage of the present invention lies in the superior toughness and resilience of the stiffening members, particularly 20 along the beveled or skived edges. These stiffening members have no inherent tendency to lose 25 their shape, are not softened to the point of distortion by ordinary temperatures of service, and are unaffected by water.

A particular advantage of the shoe stiffeners of the type employing an exuding plasticizer is 30 that their adhesiveness is not accompanied by staining of the external material of the shoe. The present compositions may readily be made colorless or light colored and hence free from the tendency which dark colored stiffeners have, 35 of imparting an undesirable graying to the delicate tints of fine fabric shoes.

When the blanks of this invention are molded from molding powder, by either injection or compression molding, there is no appreciable waste 40 or loss of material and the invention thus offers this distinct advantage in economy over the ordinary practice of cutting blanks from sheet material and beveling them by skiving which gives rise to a loss of as much as 20-30% of the sheet 45 material in the form of skeleton scrap and skivings. Also, because of the thermoplastic character of the present compositions, and the absence of reinforcing fabric and the like, any scrap that may be produced in the shaping or 50 use of the blanks of this invention (such as the sprue made in injection molding) is immediately and completely reusable.

Banks of the present material have the highly 55 essential characteristic of becoming very limp and flexible at a temperature of about 80-100° C., which is below the temperature that will cause injury to leather and, further, have the advantage of retaining this limpness, after removal of the blanks from the source of heat, for a period entirely adequate for the shaping of the blank over 60 the last. Despite the limpness and pliability of the

blanks, they are tenacious in character and can be pulled over the last without being torn. Also, as the stiffening member, after steaming, cools down toward room temperature, it still retains adequate toughness so that nails may be driven 5 through it without causing it to crack.

As many apparently widely different embodiments of this invention may be made without departing from the spirit and scope thereof, it is to be understood that the invention is not limited 10 to the specific embodiments thereof except as defined in the appended claims.

We claim:

1. A molded non-reenforced shoe stiffener blank adapted to be softened for lasting by being 15 heated to a temperature of 80-100° C., and comprising 100 parts of ethyl cellulose and 17-67 parts of plasticizer.

2. A molded, non-reenforced shoe stiffener blank adapted to be softened for lasting by being 20 heated to a temperature of 80-100° C., and comprising 100 parts of ethyl cellulose and 17-67 parts of a non-exuding plasticizer.

3. A molded, non-reenforced shoe stiffener blank adapted to be softened for lasting by being 25 heated to a temperature of 80-100° C., and comprising 100 parts of ethyl cellulose and 17-67 parts of a mixture of non-exuding and exuding plasticizers, the exuding plasticizer being present in an amount at least equal to 10% of the combined 30 weight of the ethyl cellulose and plasticizers.

4. A molded, non-reenforced shoe stiffener blank adapted to be softened for lasting by being heated to a temperature of 80-100° C., and comprising 35 100 parts of ethyl cellulose, 17-67 parts of plasticizer, and a compatible extender, said extender being present in an amount not exceeding 50% of the total weight of the composition.

5. A molded, non-reenforced shoe stiffener 40 blank adapted to be softened for lasting by being heated to a temperature of 80-100° C., and comprising 100 parts of ethyl cellulose, 17-67 parts of a non-exuding plasticizer, and a compatible 45 extender, said extender being present in an amount not exceeding 50% of the total weight of the composition.

6. A molded, non-reenforced shoe stiffener blank adapted to be softened for lasting by being heated to a temperature of 80-100° C., and comprising 50 100 parts of ethyl cellulose, 17-67 parts of a mixture of non-exuding and exuding plasticizers, the exuding plasticizer being present in an amount at least equal to 10% of the combined 55 weight of the ethyl cellulose and plasticizers, and a compatible extender, said extender being present in an amount not exceeding 25% of the total weight of the composition.

MILES C. KUMNICK.

QUENTIN L. QUINLIVAN.

60